

## UNITED STATES PATENT OFFICE.

ALFRED TINGLE, OF OTTAWA, ONTARIO, CANADA.

## PROCESS OF PRODUCING FIBER.

No Drawing.

Application filed January 25, 1924. Serial No. 688,619.

This invention relates to improved process of producing fiber, and the objects of the invention are to reduce the cost of treatment and increase the range of material, which 5 may be treated by the process involving the digestion of the raw material with aqueous solution of lime and sulphur.

Further objects are to enable the process to be carried on at such temperature and 10 under such conditions that any danger of overcooking will be avoided.

Further objects still are to provide a process to better adapt it to perform the functions required.

15 In consists essentially of the process herein described in detail in the accompanying specification.

The process is of a type involving the digestion of a fiber-producing material with 20 a solution of lime and sulphur. As a first step a raw material, which is preferably wood in a convenient form is first digested with a solution of lime and sulphur, being essentially a solution of calcium poly- 25 sulphides in water. The proportion of lime to sulphur is comparatively low, and I have found for instance, that the following proportions are satisfactory: Wood, typically in the form of spruce chips weighed in air 30 dry conditions, 100 lbs.; quicklime, 13 $\frac{1}{3}$  lbs.; sulphur (powdered finely), 6 $\frac{1}{2}$  lbs.; water, a convenient quantity up to 100 gals.

The lime, sulphur and water may be digested together before adding the wood and 35 more water, or more conveniently, the lime, sulphur and wood and water may be all digested together. The boiler used may be of steel unlined.

The temperature of digestion may range 40 from 155° C. to 170° C. The mixture is boiled under a steam pressure of 65 to 100 lbs. to the square inch, for a period of 6 to 12 hours.

The length of cooking varies according to 45 the condition and nature of the wood.

It may be observed at this point, that the action in the process is so mild, that overcooking becomes almost impossible. Thus chips such as are prepared for sulphite or 50 other digestion process may be mixed with quite fine shavings and all may be cooked together without danger of overcooking fine material in an effort to fully cook the coarser.

The product of this digestion retains most 55 of its original form and on discharge from the digester must be crushed or ground in an

edge runner, a heating engine or some similar contrivance.

It may be beaten thus with water, but a softer and superior pulp is obtained by using 60 some liquor which will largely eliminate the lime.

Such material is very various. Dilute sulphuric acid is one (1 volume of 66° Bé. acid to 10 vols. of water). Other acids 65 may be used and I prefer as cheap, convenient and productive of a good pulp, to beat with the hot waste liquor from the digestion of wood by the sulphite process. This material is commonly known as "sul- 70 phite waste liquor" and contains an acid salt of calcium, but is capable of uniting with more lime, and so largely eliminating it from the polysulphide pulp.

The pulp produced above will have a dark 75 colour, the tint depending on the details of treatment. It is however strong in fiber and long in fiber if the nature and previous treatment of the wood allows of this. Its colour can be improved by bleaching with 80 hypo-chlorites in the usual manner, but this is not recommended, as a strong dark pulp is the object aimed at—something to use in wrapping papers.

It is the less desirable to bleach this pulp 85 because it is intended to include in wood treated by this process the inner bark, discoloured shavings and such like matters at present considered refuse by most makers of pulp according to the older processes. Only 90 outer bark need be excluded, and this because it is not fibrous and thus in no case a paper making material.

In the above described process the proportion of lime to wood, lime to sulphur 95 and sulphur to wood, is much lower than in other processes of digestion with lime and sulphur, which effects a reduction in cost of the treatment, quite apart from the fact that it applies to irregular fragments of 100 wood that cannot be digested by other methods.

After digestion and grinding, the pulp is washed copiously with water and screened to remove poorly digested or badly ground 105 fragments, the resulting pulp being treated in the same way as other pulps to fit it for storage.

What I claim as my invention is:

1. A process for producing fiber, which 110 comprises digesting vegetable fiber material in an aqueous solution of lime and sulphur,

- then treating with a lime-eliminating material.
2. A process for producing fiber, which comprises digesting vegetable fiber material in an aqueous solution of lime and sulphur, then treating with an aqueous acid solution designed to eliminate lime.
3. A process for producing fiber, which comprises digesting vegetable fiber material in an aqueous solution of lime and sulphur, then treating with a sulphite waste liquor.
4. A process for producing fiber, which comprises digesting vegetable fiber material in an aqueous solution of lime and sulphur, then treating with a lime eliminating material, and then removing the colouring material from the fiber.
5. A process for producing fiber, which comprises digesting vegetable fiber material in an aqueous solution of lime and sulphur, then treating with a lime eliminating material, and then grinding the resulting material.
6. A process for producing fiber, which comprises digesting vegetable fiber material in an aqueous solution containing less than 15 per cent of lime and sulphur then treating with a lime eliminating material.
7. A process for producing fiber, which comprises digesting vegetable fiber material in an aqueous solution of lime and sulphur, then treating with a lime eliminating material, and then grinding and screening.

In witness whereof I have hereunto set my hand.

ALFRED TINGLE.